

# UNITED STATES PATENT OFFICE.

PHILIP H. MANDEL, OF ASTORIA, ASSIGNOR, BY MESNE ASSIGNMENTS, TO THE PYROPHOTO COMPANY, OF NEW YORK, N. Y.

## METHOD OF PRINTING PICTURES ON CELLULOID.

SPECIFICATION forming part of Letters Patent No. 439,533, dated October 28, 1890.

Application filed June 1, 1889. Serial No. 312,875. (No specimens.)

*To all whom it may concern:*

Be it known that I, PHILIP H. MANDEL, of Astoria, in the county of Queens and State of New York, a subject of the King of Sweden, 5 have invented certain new and useful Improvements in the Process of Printing Photographic Pictures on Celluloid, of which the following is a specification.

This invention relates to an improved process of printing photographic pictures on celluloid or other pyroxyline material and retaining them securely on the surface of the celluloid without deterioration by dampness or other causes. The photographic pictures when once fixed on the celluloid surface are permanent in color and do not fade.

The invention consists of a process of photographic printing on celluloid by first preparing the surface of the celluloid with a solution of gelatine, chrome-alum, water, and acetic acid, then transferring the picture from a tinted and sensitized paper, after the same has been exposed to the light in the negative, to the surface of the celluloid; next developing the picture on the surface of the celluloid, and, finally, hardening it by suitable chrome-alum solution and protecting the picture by a layer of suitable varnish.

The invention also consists of other features, which are hereinafter described, and specified in the claims.

In carrying out my invention the surface of the celluloid is prepared with a solution of thirty grams of gelatine, one thousand grams of water, to which a solution of one and one-half gram of chrome-alum in one hundred and sixty grams of water is added, the solution being acidulated by adding twenty grams of acetic acid.

The paper on which the photographic picture is to be produced is prepared in the following manner: It is coated with a solution of four hundred grams of water, from one hundred to one hundred and thirty grams 45 of gelatine, fifteen to twenty grams of soap, twenty to thirty grams of sugar, and four to nine grams of a suitable color, the proportion of the ingredients being varied according to

temperature. After the paper is dried the same is sensitized by a solution of thirty grams 50 of bichromate of ammonia in one thousand grams of water and a few drops of ammonia solution until the same gradually assumes a straw color. The paper is then dried in a dark room. After drying it is exposed on the negative to the action of light, requiring in the shade about five to eight minutes and in the sun from two to three minutes. After exposure the paper is placed on the celluloid surface, moistened with ice-cold water, and then 55 pressed with a rubber rule. The celluloid and paper are then subjected to pressure for about ten minutes, after which they are placed in warm water, so that the paper can be removed. The picture is then placed in a bath of cold 60 water and then dried. The last chrome-alum solution serves to fix the picture, while the treatment with warm water serves to develop the same by removing the unlighted and soluble parts of the gelatine. The picture is then 65 coated with a gelatine solution, the same gelatine solution by which the surface of the celluloid has been first coated. The picture is then hung up for drying, covered with a coating of a suitable varnish—for instance, of col- 70 lodion, consisting of equal parts of ether and alcohol, in which a small quantity of gun-cotton has been dissolved. Such a varnish unites 75 with the surface of the celluloid and forms a good protecting-layer for the picture, so that 80 the same cannot peel off or fade.

Having thus described my invention, I claim as new and desire to secure by Letters Patent—

1. The process herein described of photographing pictures on celluloid, which consists in treating the surface of the celluloid with an acidulated gelatine and chrome-alum solution, then transferring the picture from a tinted and sensitized and exposed photographic paper upon the prepared surface of the celluloid, next pressing on the picture and removing the paper, then developing and fixing the picture on the surface of the celluloid, and protecting the picture by a layer of suitable varnish, substantially as set forth. 85 90 95

2. The process of producing and securing photographic pictures on celluloid, which consists in transferring a sensitized and exposed but undeveloped photographic film onto a surface of celluloid, coated with an insoluble cement of acidulated gelatine and chrome-alum solution, and subsequently developing and fixing the same, substantially as described.

In testimony that I claim the foregoing as my invention I have signed my name in presence of two subscribing witnesses.

PHILIP H. MANDEL

Witnesses:

PAUL GOEPEL

MARTIN PETRY